

## UNITED STATES PATENT OFFICE

2,251,088

PROCESS FOR THE PRODUCTION OF ALLOYS  
CONTAINING BERYLLIUM

Helmut von Zeppelin, Bitterfeld, Germany, assignor, by mesne assignments, to Walther H. Duisberg, New York, N. Y.

No Drawing. Application August 9, 1939, Serial No. 289,177. In Germany August 26, 1937

2 Claims. (CL 75—135)

This invention relates to a process for the production of alloys containing beryllium.

Beryllium is generally alloyed with other metals by adding it in metallic form to the molten base metal whilst maintaining the melt at a temperature sufficiently high to cause dissolution of the beryllium in the base metal, and preferably whilst stirring.

It has however been observed that metallic beryllium and especially beryllium which has been obtained in the form of flakes or the like by the thermal reduction of beryllium compounds, alloys only with difficulty. It has now been ascertained that this difficulty is due to the fact that it is impossible to avoid superficial 10 oxidation of the metallic beryllium, especially in separating it from the non-metallic reaction products by lixiviation, prior to employing said beryllium for alloying purposes, the coating of oxide formed on the flakes of metallic beryllium, preventing dissolution of the beryllium by the base metal.

The present invention aims at obviating the foregoing difficulty by omitting the step of separating the metallic beryllium from the non-metallic reaction residues formed during its production.

In accordance with the invention, therefore, a mixture containing beryllium in the metallic state, which has been produced by reducing a beryllium compound with the aid of a reducing metal, is combined with the base metal to be alloyed with the beryllium in the molten state. The reducing metal employed for producing the said mixture is preferably an alkali or alkaline earth metal (including magnesium) and the reducible beryllium compound is preferably represented by a beryllium halide, especially beryllium chloride. The mixture containing beryllium in the metallic state may also contain other saline compounds, which, in a manner known per se, may be added in the production of the said mixture in order to damp the reaction and/or to lower the melting point of the non-metallic reaction residues.

In carrying out the invention there is added to the base metal with which beryllium is to be alloyed a mixture obtained by reducing a reducible beryllium compound such as beryllium chloride with a reducing metal such as magnesium and consisting substantially of metallic beryllium and the corresponding compound of the reducing metal, which mixture will hereinafter shortly be referred to as "reacted mixture."

Said reacted mixture preferably is used while

still molten and merely poured on to the molten base metal.

If the reacted mixture, preferably produced by one of the processes described in U. S. Patent No. 2,171,439 and consisting of coarsely crystalline flakes of beryllium in a magnesium chloride melt, be poured on to the molten base metal, for example copper, heated to slightly above its melting point, the beryllium alloys with the copper forthwith. The specifically lighter magnesium chloride melt floats on the metal bath during the alloying operation and in this way prevents access of air to the alloy. In consequence of the thin consistency and the low specific gravity of the magnesium chloride melt, the further advantage is obtained that the specifically heavier beryllium flakes rapidly sink down through the saline melt and thus alloy with the molten base metal bath immediately after the reacted melt is poured on to the latter.

According to still a further method of carrying out the invention, the base metal in the form of turnings or the like can be stirred into the still molten reacted mixture containing the metallic beryllium in suspension and the melt then heated up to the requisite temperature for the formation of the alloy.

The small amounts of beryllium remaining in the reacted mixture (partly in the form of oxide) 30 on completion of one of the aforementioned alloying operations can be recovered by pouring off the saline melt floating on the top of the now formed alloy, allowing it to solidify and when cold, treating it with water and finally reconverting 35 the undissolved beryllium-containing residues into beryllium chloride by chlorination.

## Example

600 parts by weight of copper, to which 3 parts by weight of magnesium had been added for deoxidation, were melted down under a thin covering of magnesium chloride. 204.5 parts by weight of a reacted mixture, produced by the reaction of beryllium chloride with magnesium and containing 25.5 parts by weight of metallic beryllium, were introduced into the melt, whilst occasionally stirring. The resulting copper-beryllium alloy, consisting of 613 parts by weight, contained 3.46% = 21.2 parts by weight of beryllium while 2.8 parts by weight of beryllium remained in the saline melt. 83% of the introduced beryllium thus alloyed with the copper, while about 11% remained in the saline melt, from which it was recovered and worked up into beryllium chloride.

I claim:

1. A process for the production of beryllium containing alloys, in which a suspension of beryllium metal in a fused non-metallic reaction residue, obtained by reaction of a beryllium halide compound with a reducing metal, is poured on to the molten base metal of the alloy to be produced.

2. A process for the production of beryllium containing alloys, in which a suspension of beryllium metal in a fused non-metallic reaction residue, obtained by reaction of beryllium chloride with magnesium is poured on to the molten base metal of the alloy to be produced.

HELMUT VON ZEPPELIN.